

Aug. 24, 1926.

1,597,571

J. BEAUDEQUIN

PROCESS FOR MANUFACTURING BRIQUETTES

Filed Nov. 29, 1924



Inventor  
d Jacques Beaudequin

By

Attala L. Morris  
Attorney

## UNITED STATES PATENT OFFICE.

JACQUES BEAUEQUIN, OF PARIS, FRANCE.

## PROCESS FOR MANUFACTURING BRIQUETTES.

Application filed November 29, 1924, Serial No. 752,976, and in Belgium December 3, 1923.

The invention relates to a process for the manufacture of combustible briquettes from carboniferous substances, such as bituminous coal or the like.

5 It has for its object more especially to enable combustible briquettes to be made of bituminous coal having the characteristics of anthracite.

The process may be best understood when 10 described in relation to apparatus by means of which it is carried out, and reference is therefore made to the sole figure of the drawing which shows, partly in plan and partly in section one form of apparatus which 15 applicant has found practical for the manufacture of briquettes according to his novel process.

In the drawing *a* represents an open-mold press into which the bituminous coal is fed 20 after having been suitably comminuted. The chamber of this press has the shape and size of a briquette, into which chamber the comminuted soft coal is fed and compressed by means of a piston, the briquettes thus 25 formed being forced into the tube *c*. This tube has the same internal diameter as the briquettes, the latter fitting tightly the bore of the tube as they are progressively forced along by successive impulses of the piston.

30 Circular metallic plates, not shown, are fed into the press between each charge of carbonaceous material, said plates being substantially of the same diameter as the internal diameter of the tube *c* and functioning 35 as separators, preventing the adherence of the briquettes one to another. The forward part of the tube *c* is heated by suitable means such as the furnace *e*, the latter, in the illustrative embodiment of the apparatus, in-

40 cluding an oven or retort *f* which surrounds the tube *c*. The column of briquettes within the tube is under considerable pressure in all directions, said pressure being transmitted by the piston of the press and being 45 resisted by the cylindrical walls of the tube and by the briquettes in the discharge end of the tube. The object of heating the briquettes while under pressure is to render viscous or liquid the hydrocarbons or coal 50 tars therein contained, to cause these to permeate the intramolecular interstices of the

briquette, transforming, in a few minutes, the bituminous coal into a coal having anthracitic qualities. At this stage in the process the metallic separators perform the 55 important function of heat conductors so that the briquettes are uniformly heated throughout to the temperature of the tube walls.

That part of the tube *d* which lies beyond 60 the furnace has a cooling function, and in this part of the tube the metallic separators serve uniformly to dissipate the heat from the briquettes, thereby inducing a gradual contraction and avoiding the cracking of 65 the briquettes which would follow their unequal cooling. It is important that the briquettes be cooled within the tube *c* and while under pressure, so that certain of the hydrocarbons which might be volatile at 70 atmospheric pressure may be condensed by the cooling of the briquette before the pressure is released.

It has been found desirable in some instances to vent the tube *c* as by the pipe *c'* 75 to permit the escape of some of the gases which are volatile throughout the entire process.

In the drawing an auxiliary press *b* has 80 been introduced, which applicant has found convenient in applying the requisite pressure to the briquettes in the tube *c*. This auxiliary press may, however, be considered as a laboratory expedient, amounting merely to a duplication of the press *a* and being entirely 85 unessential to the carrying out of the process.

What I claim and desire to protect by Letters Patent is:

1. The process for making briquettes of anthracitic quality from bituminous coal 90 which consists in forming briquettes, forcing them successively into and through a tube in a column which tightly fits the bore of said tube, heating the briquettes in a forward part of the tube while under pressure 95 to a sufficient temperature to cause fluorescence of the hydrocarbons therein contained cooling the briquettes while still under pressure in the tube.

2. The process for making briquettes of 100 anthracitic quality from bituminous coal which consists in forming briquettes, ar-

ranging conductive separators in alternation with the briquettes, forcing the briquettes successively into and through a tube in a column which tightly fits the bore of said tube heating the briquettes in the forward part of the tube while under pressure, to a sufficient temperature to cause fluorescence of the hydrocarbons therein contained, and progressively cooling the briquettes while still under pressure in the rearward part of said tube.

In testimony whereof I affix my signature.

JACQUES BEAUDEQUIN.